

# UNITED STATES PATENT OFFICE.

GEORGE BEACOCK, OF BROCKVILLE, CANADA.

## MANUFACTURE OF DRESS-STAYS.

SPECIFICATION forming part of Letters Patent No. 614,823, dated November 29, 1898.

Application filed April 29, 1898. Serial No. 679,186. (No model.)

*To all whom it may concern:*

Be it known that I, GEORGE BEACOCK, of Brockville, in the Province of Ontario, in the Dominion of Canada, have invented certain new and useful Improvements in the Manufacture of Dress-Stays, (for which I have obtained a patent in Canada, No. 59,510, dated April 4, 1898,) of which the following is a specification.

10 My invention relates to the manufacture of dress-stays from rawhide, and the object of the invention is to give to the material the required elasticity and spring to suit it to the requirements of use; and my invention consists in the treatment of the rawhide as hereinafter set forth, whereby the rawhide will be hardened and adapted to be cut into strips and finished in imitation of whalebone.

The rawhide is prepared by first placing it 20 on a table or flat surface, the hair side up, and dehaired by wetting with a solution of sulfid of sodium, to remain wet for from six to ten hours. The solution is made by dissolving the sulfid of sodium in water to be of the 25 strength from 15° to 18° Baumé. The hide is then washed and scraped and placed in a solution of borax for about six hours to toughen the hide and clean out the sodium sulfid without destroying the gelatin in the hide. The 30 solution is made by dissolving three pounds of borax in one hundred pounds of water or proportionately. The hide is then split to the thinness required for the stays and the splits immersed in any desired coloring-matter for 35 appearance. The splits are then tacked to stretchers and dried, and when dry immersed in benzin or naphtha to remove natural odors and adapt the same to receive by impregnation a waterproofing liquid which is composed 40 primarily of alcohol, gum-shellac, and rosin, with or without sulfur. The waterproofing liquid may be applied to the hide or splits with a brush, or if in large quantity by dipping into the solution or liquid. The waterproofing causes the hide to harden, and when 45

cut into strips the strips become flexible like whalebone, of which the material is a good imitation. The strips of rawhide are passed between rollers having an abrasive surface to remove inequalities and finished by passing 50 them between buffing-rollers or through a buffing-machine and then waxed to produce a polished surface.

I claim as my invention—

1. The process of preparing rawhide for the 55 manufacture of dress-stays, which consists in dehairing the hide by applying sulfid of sodium dissolved in water, then cleaning the hide by washing and scraping, then applying a solution of borax to toughen the hide and 60 remove the sodium sulfid, then splitting the hide to the thinness desired, and if preferred, staining the splits of a desired color, then stretching the splits to dry, and when dried saturating them with benzin or naphtha to remove natural and other odors, and applying a waterproofing liquid to harden the 65 hide splits, substantially as set forth.

2. The process of manufacturing dress-stays from rawhide, which consists in dehairing the 70 hide by applying a solution of sulfid of sodium and cleaning the same by washing and scraping, then applying a solution of borax to toughen the hide and remove the sodium sulfid, then splitting the hide to the thinness 75 desired, staining the splits if preferred and stretching the splits to dry, and when dried saturating them with benzin or naphtha to remove natural odors, then applying a waterproofing liquid to harden the hide splits or 80 material, then cutting the same into strips, and passing the strips between rollers having an abrasive surface and finally buffing and waxing the strips to give a finished appearance, as set forth.

GEORGE BEACOCK.

Witnesses:

JOHN GRIST,  
H. H. HORSEY.